

# UNITED STATES PATENT OFFICE.

PETER C. REILLY, OF INDIANAPOLIS, INDIANA.

## MATERIAL FOR THE PRESERVATION OF LUMBER.

1,220,001.

Specification of Letters Patent. Patented Mar. 20, 1917.

No Drawing. Application filed March 28, 1914, Serial No. 827,966. Renewed June 9, 1916. Serial No. 102,802.

*To all whom it may concern:*

Be it known that I, PETER C. REILLY, a citizen of the United States, residing at Indianapolis, in the county of Marion and State of Indiana, have invented certain new and useful Improvements in Material for the Preservation of Lumber, of which the following is a specification.

My present invention pertains to an improved material for the treatment of lumber, for the preservation thereof.

In the manufacture of such material I have, through a new process of distillation of coal tar or coal tar pitch, produced two new substances and intermixed said substances with a suitable solvent, preferably the lighter oils driven off during the first distillation of coal tar, and used this compound as a preservative material for treating lumber.

Ordinarily, in the distillation of coal tar, such distillation is discontinued when the anthracene oil stops coming over. It has been proposed heretofore in an experimental manner to continue such distillation, but according to Lunge, in "*Coal Tar and Ammonia*," 4th edition, 1909, p. 454, *et seq.*, such attempts to completely distil coal tar or coal tar pitch have not been successful.

I have by the employment of a still which is subjected to an even temperature over its entire exterior surface, been able to commercially distil coal tar and coal tar pitch so that they will ultimately produce three products heretofore not commercially known, namely, a material orange in color which passes from the still when the same is subjected to a temperature approximately from 700° to 800° F., this after the anthracene has passed over, which material is waxy at 70° F., and has a specific gravity of from 1.147 up to 1.22; secondly, a hard, garnet-colored product, brittle at 70° F., having a specific gravity of not less than 1.22 and which, when cut with a knife flakes, the cut surface of the material likewise being of a brilliant garnet color; and thirdly, a dry coke, sponge-like in appearance and which is readily handled. These

first two products I intermix and dissolve in a suitable solvent such, for instance, as the oils distilled from coal tar during the first distillation thereof. The mixture thus produced is extremely valuable for use in

the preservation of wood, and lumber, such as street-paving materials, railroad ties and the like. Heretofore the relatively light oils produced in the distillation of coal tar have been employed as preservatives for lumber, but inasmuch as they have a very low boiling-point and are of a specific gravity not much higher than that of water, they rapidly escape from the timber by volatilization and are to a slight extent washed away by water. When, however, such oils are mixed with the heavy products above mentioned this does not occur. After being once passed into the material, the mixture remains therein, regardless of temperature or moisture conditions, the compound being very efficient as a preservative and likewise being stable. The dry coke above mentioned does not, of course, enter into the preservative composition, but is employed in various commercial ways.

No claim is made herein to the process of producing the materials above set forth, as that forms the subject matter of my pending application Serial No. 827,965, filed on or about March 28, 1914, nor is any claim made to the still which is subject to an even temperature over its entire exterior surface, as above mentioned, as said still construction forms the subject matter of my pending application Serial No. 827,967, filed on or about March 28, 1914.

Having thus described my invention, what I claim is:

1. A composition of matter, for use in the preservation of timber, comprising a mixture of waxy material produced as a distillate from coal tar, and having a specific gravity of not less than 1.14; a hard material formed as a distillate from coal tar and having a specific gravity of not less than 1.22; and a suitable solvent for said materials.

2. A composition of matter, for use in the preservation of timber, comprising a mixture of a waxy material produced as a distillate from coal tar, and having a specific gravity of not less than 1.14; and a hard material formed as a distillate from coal tar and having a specific gravity of not less than 1.22, said materials being dissolved in the lighter oils distilled from coal tar.

3. A composition of matter, for use in the preservation of timber, comprising a mix-

ture of those materials which are produced as a distillate from coal tar when the latter is subjected to a temperature of at least 700° F., said material having a specific gravity in excess of 1.14, said distillates being dissolved in a suitable solvent.

4. A composition of matter for the treatment of timber, comprising a mixture of all of the distillates of coal tar which are driven

off therefrom up to a temperature approxi- 12  
mating 1000° F.

In testimony whereof I have signed my name to this specification in the presence of two subscribing witnesses.

PETER C. REILLY.

Witnesses:

HORACE A. DODGE,  
BENNETT S. JONES.